

# UNITED STATES PATENT OFFICE.

MILTON C. WHITAKER, OF NEW YORK, N. Y., ASSIGNOR TO U. S. INDUSTRIAL ALCOHOL CO., A CORPORATION OF WEST VIRGINIA.

## FUEL ADAPTED FOR USE IN INTERNAL-COMBUSTION ENGINES.

1,423,058.

Specification of Letters Patent. Patented July 18, 1922.

No Drawing.

Application filed November 12, 1919. Serial No. 337,398.

To all whom it may concern:

Be it known that I, MILTON C. WHITAKER, a citizen of the United States, residing at New York, in the county of New York and State of New York, have invented a certain new and useful Improvement in Fuels Adapted for Use in Internal-Combustion Engines, of which the following is a specification.

10 My invention relates particularly to fuels designed to be used in any desired manner, but it has application especially to fuels adapted to be used as a source of power, as for example motor fuels.

15 The object of my invention is to provide fuels containing an alcohol and an ester, which may be used for any purpose, but which are especially adapted for use in internal combustion engines, as, for example 20 aeroplane motors.

Another object of my invention is to provide a fuel containing an alcohol and a hydrocarbon, the same being blended by the presence of an ester, preferably a volatile ester as for example ethyl acetate.

Another object of my invention is to provide a motor fuel having such a large percentage of a very volatile constituent as to render the operation of aeroplane motors 30 using the same entirely certain, even at the highest altitudes reached by aeroplanes.

A further object of my invention is to provide a fuel that will not freeze, and the constituents of which will not separate 35 out at any atmospheric temperature, so that aeroplanes may be driven therewith at any desired altitude and at any desired longitude of the earth without affecting the fuel adversely. Still a further object of my 40 invention is to provide fuels of the above character containing alcohol and a petroleum hydrocarbon blended by the use of benzol.

Further objects of my invention will appear from the detailed description thereof contained hereinafter.

While my invention is capable of being carried out in different ways, for the purpose of illustration I shall describe only 50 certain ways of carrying out the same herein.

For example, a fuel made in accordance with my invention may be comprised of—

60 parts by volume of ethyl alcohol,  
55 40 parts by volume of ethyl acetate.

The percentages of the above constituents may vary to some extent, if desired. For example, the alcohol may vary from 50% to any higher percentage but preferably not amounting to 80%, and the ethyl acetate 60 may vary from any percentage above 20% up to 50%, although I have obtained the best results by the specific composition above given.

The ethyl alcohol in the above composition may be ordinary alcohol having a strength of 95%, but, preferably, I use alcohol substantially free from water, that is to say having a strength of 98% or higher, or absolute alcohol, that is alcohol having a 70 strength of at least 99%.

As another example of my invention, I may provide a fuel comprised of—

45 parts by volume of ethyl alcohol,

35 parts by volume of gasoline having a 75 specific gravity of from 52° Bé. to 66° Bé.,  
20 parts by volume of ethyl acetate.

The percentages of the above constituents may vary to some extent, if desired. For example, the ethyl alcohol may vary 80 from 30 to 60%, the gasoline may vary from 25 to 50%, and the ethyl acetate may vary from 10 to 25%, although I have obtained the best results by the specific composition above given.

Again another example of my invention may be a fuel comprised of—

25 parts by volume of ethyl alcohol,

25 parts by volume of kerosene,

25 parts by volume of gasoline,

11 parts by volume of ethyl acetate.

It is to be understood, also, that, instead of the gasoline and kerosene referred to in the above example, I may use merely gasoline.

As another example, I may make a fuel containing—

40 parts by volume of ethyl alcohol,

30 parts by volume of benzol,

30 parts by volume of gasoline or naphtha 100 having a specific gravity of from 52° to 66° Bé.,

5 parts by volume of ethyl acetate.

The percentages of the above constituents may vary to some extent, if desired. For 105 example, the alcohol may vary from 40 to 60%, the benzol from 25 to 35%, the gasoline or naphtha from 30 to 50%, and the ethyl acetate may range in percentage from 5 to 20%, although I have obtained the best re- 110

sults by the specific composition above given.

By the use of the ethyl acetate in this composition I avoid the necessity of using alcohol having a greater strength than 95%, as the ethyl acetate itself will prevent the benzol from crystallizing out at very low temperatures.

Instead of the benzol, furthermore, I may use toluol.

10 Further examples of my invention may be fuels containing the following constituents, the characteristics of which are that they contain hydrocarbons and alcohol, as well as an ester, but will not freeze or separate 15 out under atmospheric temperatures:

40 parts by volume of ethyl alcohol,  
28 parts by volume of gasoline,  
17 parts by volume of benzol,  
7.5 to 10 parts by volume of ethyl acetate,  
20 8 parts by volume of toluol.

Another example is the following:  
20 parts by volume of ethyl alcohol,  
20 parts by volume of gasoline,  
15 parts by volume of kerosene,  
25 35 parts by volume of methyl-ethyl-ketone,  
5 parts by volume of ethyl acetate.

Another example is:  
15 parts by volume of benzol,  
40 parts by volume of alcohol,  
30 30 parts by volume of gasoline,  
15 parts by volume of ethyl acetate.

Compositions of the above character will not freeze within the range of the usual atmospheric temperatures, as for example, a 35 temperature as low as minus 50° F., nor even down to a temperature of minus 60° F. By atmospheric temperatures I mean temperatures down to minus 50° F.

The toluol is especially advantageous in 40 preventing the freezing of such compositions and particularly where benzol is used as the blending agent.

In all the above compositions any desired 45 alcohol may be used, such for example as methyl alcohol, ethyl alcohol, butyl alcohol, etc., but I prefer to use ethyl alcohol, and the number of parts thereof in the above compositions may vary to a considerable extent. The alcohol used in any of the above 50 compositions may be ordinary alcohol having a strength of 95%, but I may use an alcohol having a greater strength, which may even be absolute alcohol. Instead of

the ethyl acetate, I may use any one of a number of other esters, as for example 55 methyl butyrate, ethyl butyrate, methyl acetate, butyl acetate or amyli acetate, all of which are volatile esters or still other esters could be used as for example, castor oil.

Also, the proportion of the ester present 60 may vary to a considerable extent. Furthermore, instead of the gasoline other hydrocarbons may be used, and the range of the proportions of the same in the above compositions may vary to a considerable extent. 65 Different blending agents may be used which are of such a character as to blend the above constituents, but which will also not produce a composition that would freeze at atmospheric temperatures. 70

While I have described my invention above in detail, I wish it to be understood that many changes may be made therein without departing from the spirit thereof.

I claim:

1. A fuel comprising an alcohol above 20 parts by volume, benzol 17 to 35 parts, gasoline 20 to 50 parts, and ethyl acetate 5 to 20 parts.

2. A fuel comprising an alcohol above 20 parts by volume, benzol 17 to 35 parts, gasoline 20 to 50 parts, ethyl acetate 5 to 20 parts, and toluol.

3. A fuel comprising ethyl alcohol 40 parts by volume, gasoline 28 parts, benzol 85 17 parts, ethyl acetate 7½ to 10 parts, and toluol 8 parts.

4. A fuel comprising an alcohol above 20 parts by volume, gasoline 20 to 50 parts, and ethyl acetate 5 to 20 parts. 90

5. A fuel comprising an alcohol above 20 parts by volume, gasoline 20 to 50 parts, ethyl acetate 5 to 20 parts, and toluol.

6. A fuel comprising an alcohol above 20 parts by volume, an aromatic hydrocarbon 95 17 to 35 parts, a petroleum distillate 20 to 50 parts, and an ester 5 to 20 parts.

7. A fuel comprising ethyl alcohol above 20 parts by volume, an aromatic hydrocarbon 17 to 35 parts, gasoline 20 to 50 parts, and 100 an ester 5 to 20 parts.

In testimony that I claim the foregoing, I have hereunto set my hand this 6th day of November, 1919.

MILTON C. WHITAKER.